

# UNITED STATES PATENT OFFICE.

HILAIRE DE CHARDONNET, OF BESANCON, FRANCE.

## PROCESS OF DYEING ARTIFICIAL SILK.

SPECIFICATION forming part of Letters Patent No. 410,404, dated September 3, 1889.

Application filed June 22, 1888. Serial No. 277,895. (No specimens.) Patented in France January 27, 1888, No. 188,304, and in England April 9, 1888, No. 5,270.

*To all whom it may concern:*

Be it known that I, HILAIRE DE CHARDONNET, a citizen of the Republic of France, and a resident of Besançon, (Doubs,) France, have 5 invented certain new and useful Improvements in the Art of Denitrating and Dyeing Artificial Silk and other Pyroxylene Substances, (which invention is the subject of Letters Patent in France No. 188,304, dated January 27, 1888, and in England, No. 5,270, dated April 9, 1888,) of which the following is a specification.

When a pyroxylene in filaments or in sheets molded in different ways is digested in a 15 bath containing certain reducing substances, as sugar, acetic acid, alcohol, protochloride of iron, &c., and when likewise pure water is employed, the pyroxylene is seen to gradually lose under the influence of time and temperature its combined nitrogen. Nitric acid produces the same effect in a more regular and 20 complete manner. The action is increased by direct reason of the length of time, the concentration, and the temperature, which may 25 vary within wide limits, all leading to the desired result.

The process of denitration which I have invented is the following: The pyroxylene is maintained at 30° to 35° centigrade in a 30 bath of nitric acid of a density of about 1.32. In a few hours it loses a part of its nitrogen and descends beneath the tetranitric cellulose (Mr. Vieille.) This transformation is recognized either by an analysis or by a test 35 of the solubility, or by observing at the beginning the softening which the pyroxylene undergoes. It is then washed rapidly with tepid or cold water, then dipped at this moment in the dyeing-bath, then washed with 40 cold water, and dried in a current of tepid air.

This process applied to artificial silk (spun collodion) dispenses with the introduction into the mother solution of metallic chlorides 45 and alkaloids, (designed to reduce the combustibility.)

The results which I have obtained lead me

to the conclusion that the action is as follows: The bath of nitric acid tends, according to its concentration, to establish a chemical equilibrium between the affinity of the cellulose and the affinity of the water for the nitric acid—an equilibrium which varies continually according to the temperature, the nitration, and the density of the acid. The cellulose 55 may charge itself with nitric acid at all degrees from zero up to seventy-five or eighty per centum, whether the combination is in definite proportions or not.

I give below a table of the results of an 60 analysis of the reaction:

| Time.                     | Cubic centimeters of nitrogen dioxide liberated from 0.5 gram of pyroxylene. | Milligrams of nitrogen contained in one gram of pyroxylene. | Milligrams of nitric acid contained in one gram of pyroxylene. |    |
|---------------------------|------------------------------------------------------------------------------|-------------------------------------------------------------|----------------------------------------------------------------|----|
| Before the operation..... | 90                                                                           | 113                                                         | 435                                                            | 65 |
| At end of 1 hour.....     | 88                                                                           | 110                                                         | 434                                                            |    |
| At end of 3 hours.....    | 82                                                                           | 103                                                         | 399                                                            |    |
| At end of 6 hours.....    | 64                                                                           | 80                                                          | 310                                                            |    |
| At end of 7 hours.....    | 55                                                                           | 68                                                          | 264                                                            | 70 |
| At end of 7½ hours.....   | 50½                                                                          | 63                                                          | 244                                                            | 75 |

I claim as my invention—

The process of dyeing artificial silk and other pyroxylene compounds, which consists in, first, denitrating the artificial silk or pyroxylene compound by immersion for a few hours in a bath of nitric acid; second, washing the denitrated material, and, third, dipping the same in a dyeing-bath, substantially 85 as set forth.

In witness whereof I have hereunto signed my name in the presence of two subscribing witnesses.

HILAIRE DE CHARDONNET.

Witnesses:

ROBT. M. HOOPER,  
AMAND RITTER.